

## UNITED STATES PATENT OFFICE

2,296,238

## CARBURETED EMISSIVE ELECTRODE

Jean Baptiste Joseph Marcel Abadie,  
Puteaux, FranceNo Drawing. Application January 22, 1940,  
Serial No. 315,018

1 Claim. (CL 176—126)

This invention is directed to electrodes for discharge tubes and a method of making them. More specifically, the invention relates to the production of activated electrodes comprised generally of a metal support containing an electron emissive coating.

Briefly, the present invention is predicated upon the employment of a carbureted alkaline earth metal or salt as an electron emissive electrode coating. Such electrodes act suitably either as anodes or cathodes, and it has been discovered that the carbon which enters into the constitution of the electrodes imparts to them the thermic inertia necessary to their proper operation as cathodes. Typical spot formations seen frequently on the glass walls of tubes or lamps filled with mercury vapor after continued operation do not occur when the electrodes of the present invention are employed in such tubes. The electrodes furthermore are suited particularly for use in the quantity production of gaseous discharge tubes, sodium lamps, luminescent rare gas tubes operating upon either high or low voltages, or relatively high pressure metallic vapor lamps.

In the practice of the present invention, an electrical conductive support is employed for carrying the carbide layer. This support may be comprised of nickel, molybdenum, tungsten or carbon. The support may be in the form of a cup or crucible spiral wire, or plate or the like, suitably arranged to carry the emissive coating.

One of the most convenient means for forming the carbide layer is as follows: To anhydrous baryta is added from approximately 20 to 40% by volume of quicklime. Water is added to this mixture to form a somewhat syrupy sludge and then the electrically conductive support is dipped into this sludge and dried, either in an oven or in an open flame. The temperature attained during the drying should not, generally speaking, be higher than that of a dull red; if the temperature exceeds this range there is danger of volatilization of the coating material applied to it. The primary purpose in drying the coating is to harden it upon its support.

The metal support may be dipped once, or a number of times if a coating of increased thickness is desired. It is recommended that each layer of coating be dried and hardened in order that a layer of increased thickness cumulatively be built upon the support material.

After a coating of the desired thickness has been obtained upon the metal support, the electrode next is dipped into a mixture containing graphite or finely divided carbon. The carbon or graphite may either be held in suspension or may be in such mixture as to produce a coating

after carbonization. For instance, a mixture made of approximately equal parts of graphite and sugar is suitable, with enough water added to obtain a syrupy composition. After the electrode has been dipped in the graphitic mixture it is allowed to dry slightly and it is then heated in a flame so that the sugar is carbonized and the water evaporated.

10 A single coating operation in place of the double coating operation may be followed if desired. For example, the conductive support may be treated once or a number of times and dried, as described, in a mixture comprised of approximately  $\frac{2}{3}$  of a mixture of equal parts of graphite and sugar and  $\frac{1}{3}$  of a mixture of lime and baryta, enough water again being used to provide a sludge or syrup sufficiently fluid to facilitate the application of the coating to the support.

20 The alkali or alkaline earth carbides are formed in the electrode during the pumping operation. In this way the carbon enters into the constitution of the electrode.

25 During the pumping operation the presence of the carbon causes an extremely rapid production of the emissive salts used. For instance, in a typical operation a current is passed through the tube during the period that it is being pumped, the salts are reduced, carbides are formed and the electrodes are purified and ready for usage in the tube in which they are to be contained.

30 In place of the lime and baryta used for constituting the electrode other alkaline earth salts may be employed either alone or in conjunction with alkali metal salts.

35 The carbon contained in the electrodes has a very high anodic drop in rare gases as well as in metallic vapors.

40 The electrodes are characterized particularly in that carbon in the powdery form is associated with the emissive metal in the form of a coating over the electrically conductive support, and in that the electrodes so constituted may be used indifferently as cathodes or anodes in gaseous discharge tubes.

45 Having described my invention, I claim:

An electrode for a discharge tube which is characterized in that it may be used indifferently as a cathode or an anode and which is comprised of an electrically conductive support containing a coating comprised of an emissive material selected from the group consisting of alkaline earth metals and alkaline earth salts intimately associated with powdered carbon which is physically present as free carbon.

JEAN BAPTISTE JOSEPH  
MARCEL ABADIE,